

## UNITED STATES PATENT OFFICE

2,291,021

## CELLULOSIC MATERIAL

Louis H. Bock, Glen-side, and Alva L. Houk, Philadelphia, Pa., assignors to Rohm & Haas Company, Philadelphia, Pa.

No Drawing. Application July 31, 1940,

Serial No. 348,829

## 15 Claims.

This invention concerns the improvement of cellulosic materials, particularly cellulosic fibers, and is based on the reaction of cellulosic materials with aldehydo quaternary ammonium compounds of the general formula



wherein  $\text{R}$  is an aliphatic, arylaliphatic, or hydroarylaliphatic group having at least one hydrogen on the carbon atom attached to the ether oxygen atom,  $\text{R}_1$  and  $\text{R}_2$  are members of the class consisting of aliphatic groups and cycloaliphatic hydrocarbon groups when taken singly and when taken together divalent saturated aliphatic radicals which jointly with the nitrogen form a heterocycle,  $\text{R}_3$  is a member of the group consisting of hydrogen and alkyl groups,  $\text{R}_4$  is a member of the class consisting of hydrogen and aliphatic hydrocarbon groups and  $\text{X}$  is a halogen.

We have described in application Serial No. 309,398, filed December 15, 1939, how polysaccharides may be rendered resistant to the usual action of water by treating them with the acid salt of an aminomethyl aldehyde. We have now found that the aldehydo quaternary ammonium compounds of the above formula are even more effective in rendering cellulose water-resistant so that swelling of cellulose in films or fibers and changes in dimension of cellulose fabrics are minimized without loss of the essential fundamental properties thereof or change in general appearance.

Treating cellulosic textile materials with a solution of an aldehydo quaternary ammonium compound of the above formula and heating the treated material above about 100° C. causes a reaction to occur between some of the hydroxyl groups of the cellulose and the aldehydo quaternary compound. Thereby the nature of the cellulose is superficially changed. If a group added from the aldehydo quaternary ammonium compound possesses a long hydrocarbon chain, the surface of the cellulosic material is rendered water-repellent. If the groups are small, the replacement of hydroxyl groups nevertheless renders the cellulosic material sufficiently hydrophobic to decrease the sensitivity of the material to water. As a result of the reaction, therefore, cellulosic fabrics become more stable in dimensions than untreated fabric.

The aldehydo quaternary ammonium compounds of the above formula are obtained as de-

(CL. 8—116)

scribed in application Serial No. 350,134, filed August 2, 1940, by reacting a disubstituted aminomethyl aldehyde of the formula



with a halomethyl ether of a primary or secondary alcohol, having the formula  $\text{ROCH}_2\text{X}$ , where the symbols have the same significance as above. The aminomethyl aldehydes are formed by reacting such aldehydes as acetaldehyde, propionaldehyde, isobutyraldehyde, valeraldehyde, dodecylaldehyde, 9,10-octadecenylaldehyde, octadecylaldehyde, etc. with formaldehyde and a reactive amine such as dimethylamine, dibutylamine, diethylamine, caprylmethylamine, methylcyclohexylamine, dicyclohexylamine, morpholine, piperidine, etc. The halomethyl ethers are obtained from such alcohols as methyl, ethyl, butyl, octyl, dodecyl, octadecyl, allyl, undecenyl, 9,10-octadecenyl, capryl, dicapryl, benzyl, hexahydrobenzyl, phenoxyethyl, etc. by reacting them with formaldehyde and hydrogen chloride.

Typical of the aldehydo quaternary ammonium halides which may be prepared are the following:



Ethoxymethyl dimethyl  $\beta$ -methyl- $\beta$ -formyl-propyl ammonium chloride



Butoxymethyl dimethyl  $\beta$ -methyl- $\beta$ -formyl-propyl ammonium chloride



Capryloxymethyl  $\beta$ -formyl-ethyl diethyl ammonium chloride



Allyloxymethyl  $\beta$ -formyl-propyl piperidinium chloride

Phenoxyethoxymethyl  $\beta$ -formyl-propyl morpholinium chlorideButoxymethyl dimethyl  $\beta$ -formyl-octadecyl ammonium chloride

Typical cellulosic textile materials include cotton, linen, regenerated cellulose, cellulose esters, cellulose ethers, etc. in the form of fibers, filaments, films, sheets, yarn, fabric. In this invention the use of any cellulosic textile material having free hydroxyl groups is contemplated.

The cellulosic material is treated with the aldehydo quaternary ammonium compound preferably in solution in water or an organic solvent. Solutions having concentrations from 1% to about 10% are particularly suitable. When fabric, yarn, fibers, etc. are passed through a solution, sufficient of the compound is absorbed or adsorbed to react with sufficient hydroxyl groups to overcome hydrophilic tendencies yet without degrading or disintegrating the treated material.

The following examples illustrated the modification of cellulose with the aldehydo quaternary ammonium compounds.

#### Example 1

A piece of 80 x 80, 4 yd., 36 in. cotton sheeting was firmly clamped in a rigid frame and impregnated with a 10% aqueous solution of the quaternary ammonium salt obtained from 2-ethyl hexoxymethyl chloride and dimethylaminoneopental (2-ethyl hexoxymethyl dimethyl  $\beta$ -methyl- $\beta$ -formyl-propyl ammonium chloride). The cloth was dried at room temperature and then heated for one-half hour at 130° C. while still in the frame. The piece of cloth was removed from the frame and carefully measured. It was then laundered in a hot solution of soap and soda ash, rinsed, dried, and ironed. The dimensions of the piece of cloth were again determined. Shrinkage in the direction of the warp was 2.3%. The shrinkage of the original sheeting subjected to the same laundering process was 5.25%.

#### Example 2

Another piece of the same cotton sheeting was treated according to the procedure described in Example 1, except that there was used a 10% aqueous solution of the quaternary ammonium salt obtained from benzyloxymethyl chloride and diethylaminoneopental (benzyloxymethyl diethyl  $\beta$ -methyl- $\beta$ -formyl-propyl ammonium chloride). Shrinkage along the warp direction was 1.96%.

#### Example 3

Another piece of the cotton sheeting was impregnated with a 10% aqueous solution of methallyloxymethyl dimethyl  $\beta$ -formyl- $\beta$ -methyl-propyl ammonium chloride, following the same general procedure as described in Example 1. The dried, impregnated fabric was heated for 35 minutes at 120-130° C. After the dimensions of the treated cloth had been determined, the cloth was laundered as in Example 1. It was then found that shrinkage warp-wise was 0.98%.

5

10

15

20

25

30

35

40

45

50

55

57

60

65

67

70

75

#### Example 4

A piece of the sheeting used in the above examples was clamped in the frame, immersed in a 10% aqueous solution of dodecyloxymethyl dimethyl  $\beta$ -methyl- $\beta$ -formyl-propyl ammonium bromide, dried for five minutes in an oven at 127° C., and then heated in an oven at 150° C. for five minutes. The cloth was removed from the frame and laundered as in the preceding examples. Shrinkage along the warp was now only 1.84%.

#### Example 5

A piece of the cotton sheeting already described was padded through a 5% aqueous solution of the quaternary ammonium salt obtained by reacting butoxymethyl chloride and  $\alpha$ -dimethylaminomethyl octadecylaldehyde. The cloth was dried at room temperature and then baked in an oven at 120° C. for 30 minutes. The cloth was highly repellent to water. It was then laundered with a solution of soap and soda ash, rinsed carefully, dried, and ironed. The repellency was still very high.

#### Example 6

The procedure of Example 5 was followed with a piece of spun rayon fabric. The treating agent was octadecyloxymethyl dimethyl  $\beta$ -methyl- $\beta$ -formyl-propyl ammonium chloride. The treated cloth likewise possessed a water-repellent finish which was fast to laundering.

#### Example 7

Kraft paper was impregnated with a 20% solution of dodecyloxymethyl dimethyl  $\beta$ -methyl- $\beta$ -formyl-propyl ammonium chloride. It was then placed in an oven at 140° C. for forty minutes. The resulting paper had an increased resistance to disintegration by water.

#### Example 8

Example No. 1 was repeated using cotton yarn. The resistance to shrinkage was greatly improved.

The treating of cellulosic materials with an aldehydo quaternary ammonium halide followed by heating to cause a reaction between the cellulosic material and the halide yields a product which is less sensitive to water than untreated material. Woven fabric becomes resistant to changes in dimensions during washing. This effect may be utilized in conjunction with a mechanical shrinking procedure to give superior, shrunk fabrics. If desired, the process of this invention may be adapted to altering the surface of cotton, rayon, linen, and the like so that fabrics of these materials shed water. The reaction of long-chained groups with cellulose gives a softening effect which is permanent.

We claim:

1. A method for improving cellulosic textile materials having free hydroxyl groups which comprises treating said materials with a solution of a compound having the formula



wherein R is a member of the class consisting of aliphatic, arylaliphatic, and hydroarylaliphatic groups having at least one hydrogen on the carbon atom attached to the ether oxygen atom, R1 and R2 are members of the class consisting of aliphatic groups and aliphatic hydrocarbon

groups when taken singly and when taken together divalent saturated aliphatic radicals which jointly with nitrogen form a heterocycle, R<sub>3</sub> is a member of the class consisting of hydrogen and alkyl groups, R<sub>4</sub> is a member of the class consisting of hydrogen and aliphatic hydrocarbon groups, and X is a halogen, and heating the treated materials between 100° C. and about 150° C.

2. A method for improving cellulosic textile fibers having free hydroxyl groups, which comprises treating said fibers with a solution of a compound having the formula



wherein R is a member of the class consisting of aliphatic, arylaliphatic, and hydroarylaliphatic groups having at least one hydrogen on the carbon atom attached to the ether oxygen atom, R<sub>3</sub> is a member of the class consisting of hydrogen and alkyl groups, and R<sub>4</sub> is a member of the class consisting of hydrogen and aliphatic hydrocarbon groups, and heating the treated materials between about 100° C. and the decomposition temperature of the cellulosic material.

3. A method for increasing the water-resistance of cotton which comprises treating cotton with a solution of a compound having the formula



wherein R is an aliphatic, hydrocarbon group having at least one hydrogen atom on the carbon atom attached to the ether oxygen atom, R<sub>3</sub> is a member of the class consisting of hydrogen and alkyl groups, and R<sub>4</sub> is a member of the class consisting of hydrogen and aliphatic hydrocarbon groups, and heating the cotton between about 100° C. and about 175° C.

4. A method for increasing the water-resistance of cellulosic textile fibers having free hydroxyl groups, which comprises treating said fibers with a solution of a compound having the formula



wherein R is a member of the class consisting of aliphatic, arylaliphatic and hydroarylaliphatic groups having at least one hydrogen on the carbon atom attached to the ether oxygen atom, R<sub>3</sub> is a member of the class consisting of hydrogen and alkyl groups, and R<sub>4</sub> is a member of the class consisting of hydrogen and aliphatic hydrocarbon groups, at least one of the groups R and R<sub>4</sub> having more than 12 carbon atoms, and heating the treated materials between about 100° C. and the decomposition temperature of said cellulosic fibers.

5. A method for increasing the water-resistance of cellulosic textile fibers having free hydroxyl groups, which comprises impregnating said fibers with a solution of an alphyoxymethyl dimethyl  $\beta$ -methyl- $\beta$ -formyl-propyl ammonium chloride and heating the treated fibers above 100° C. but below the decomposition temperature of said fibers.

6. A method for imparting hydrophobic properties to cellulosic textile fibers having free hy-

droxyl groups, which comprises impregnating said fibers with a solution of a dodecyloxymethyl dimethyl  $\beta$ -formyl- $\beta$ -methyl-propyl ammonium chloride and heating the treated fibers above 100° C. but below the decomposition temperature of said fibers.

7. A method for increasing the water-resistance of cellulosic textile fibers having free hydroxyl groups, which comprises impregnating said fibers with a solution of a butoxymethyl dimethyl  $\beta$ -formyl-octadecyl ammonium chloride and heating the treated fibers above 100° C. but below the decomposition temperature of said fibers.

8. A method for stabilizing a woven cellulosic fabric which comprises impregnating said fabric with a solution of a butoxymethyl dimethyl  $\beta$ -formyl- $\beta$ -methyl-propyl ammonium halide and heating the impregnated fabric above 100° C. but below the decomposition temperature of said fabric.

9. Hydroxyl-bearing cellulosic textile materials having hydroxyl groups reacted with a compound of the formula



wherein R is an aliphatic, arylaliphatic, or hydroarylaliphatic group having at least one hydrogen on the carbon atom attached to the ether oxygen atom, R<sub>1</sub> and R<sub>2</sub> are members of the class consisting of aliphatic groups and cycloaliphatic hydrocarbon groups when taken singly

35 and when taken together divalent saturated aliphatic radicals which jointly with the nitrogen form a heterocycle, R<sub>3</sub> is a member of the group consisting of hydrogen and alkyl groups, R<sub>4</sub> is a member of the class consisting of hydrogen and 40 aliphatic hydrocarbon groups and X is a halogen.

10. Hydroxyl-bearing cellulosic textile materials having hydroxyl groups reacted with a compound of the formula



wherein R is an aliphatic hydrocarbon group, having at least one hydrogen atom on the carbon atom attached to the ether oxygen atom, R<sub>3</sub> is a member of the class consisting of hydrogen and alkyl groups, and R<sub>4</sub> is a member of the class consisting of hydrogen and aliphatic hydrocarbon groups.

11. Hydroxyl-bearing cellulosic textile material having hydroxyl groups reacted with a butoxymethyl dimethyl  $\beta$ -formyl-octadecyl ammonium halide.

12. Hydroxyl-bearing cellulosic textile material having hydroxyl groups reacted with a dodecyloxymethyl dimethyl  $\beta$ -formyl- $\beta$ -methyl-propyl ammonium halide.

13. Hydroxyl-bearing cellulosic textile material having hydroxyl groups reacted with a butoxymethyl dimethyl  $\beta$ -formyl- $\beta$ -methyl-propyl ammonium halide.

14. Woven cotton textile fabric having hydroxyl groups reacted with a compound of the formula



75 wherein R is an aliphatic hydrocarbon group

having at least one hydrogen atom on the carbon atom attached to the ether oxygen atom,  $R_3$  is a member of the class consisting of hydrogen and alkyl groups, and  $R_4$  is a member of the class consisting of hydrogen and aliphatic hydrocarbon groups.

15. Regenerated cellulose fabric having hydroxyl groups reacted with a compound of the formula



wherein  $R$  is an aliphatic hydrocarbon group having at least one hydrogen atom on the carbon atom attached to the ether oxygen atom,  $R_3$  is a member of the class consisting of hydrogen and alkyl groups, and  $R_4$  is a member of the class consisting of hydrogen and aliphatic hydrocarbon groups.

LOUIS H. BOCK,  
ALVA L. HOUK,